

## UNITED STATES PATENT OFFICE.

HANS RATHSBURG, OF FURTH, GERMANY.

## EXPLOSIVE COMPOUND FOR PRIMERS AND DETONATORS.

No Drawing.

Application filed August 22, 1921. Serial No. 494,386.

To all whom it may concern:

Be it known that I, HANS RATHSBURG, a citizen of the Republic of Germany, residing at Furth, in Bavaria, Germany, have invented certain new and useful Improvements in Explosive Compounds for Primers and Detonators, of which the following is a specification.

This invention relates to a new and improved initial primer or detonator and to a process for its manufacture. It is well known that fulminate of mercury hitherto employed in primers or detonators has many disadvantages. Among others it has a destructive influence upon aluminium, it is easily deadened by pressure, it is very uncertain in its action, especially at the low temperatures of liquid air, and it soon deteriorates when stored in damp places. Substitutes for fulminate of mercury which have recently been employed are likewise not free from objections.

It has now been found that the salts of tetrazole ( $\text{CH}_2\text{N}_4$ ), and its derivatives, owing to their properties, are capable of replacing fulminate of mercury and other initial explosives hitherto employed either entirely or partly, according to the object for which they are employed. The most suitable substances are: the alkali, the earthy alkali, and the heavy metal salts of tetrazole, ( $\text{CH}_2\text{N}_4$ ), tetrazoleazoimid or diazotetrazoleimid ( $\text{CHN}_7$ ), a zotetrazole ( $\text{C}_2\text{H}_2\text{N}_{10}$ ), oxyazotetrazole ( $\text{C}_2\text{H}_2\text{ON}_{10}$ ), diazoaminotetrazole ( $\text{C}_2\text{H}_3\text{N}_{11}$ ), diazotetrazole ( $\text{CN}_6$ ), bistetrazole ( $\text{C}_2\text{H}_2\text{N}_8$ ), furthermore the salts of phenyltetrazolecarbon-acid ( $\text{C}_8\text{H}_6\text{O}_2\text{N}_4$ ), methylmercaptotetrazole ( $\text{C}_2\text{H}_4\text{N}_4\text{S}$ ), substituted dioxytetrazoles, as phenethyldioxytetrazol ( $\text{C}_5\text{H}_8\text{O}_2\text{N}_4$ ), B-naphthyldioxytetrazol ( $\text{C}_{11}\text{H}_8\text{O}_2\text{N}_4$ ), phenylglycolendioxytetrazole ( $\text{C}_8\text{H}_8\text{O}_3\text{N}_4$ ), and also benzylyldioxytetrazol ( $\text{C}_7\text{H}_6\text{O}_2\text{N}_4$ ), meta-nitrobenzylyldioxytetrazol ( $\text{C}_7\text{H}_5\text{O}_4\text{N}_5$ ), para-tolenyldioxytetrazole ( $\text{C}_8\text{H}_8\text{O}_2\text{N}_4$ ), as well as similar derivatives and substitution products of tetrazole. The salts of the stable triazole, as in Beilsteins "Handbuch der Organischen Chemie" 3rd ed. vol. 4, page 1098, may also be employed.

As some of the referred to substances are of recent discovery, attention is directed to applicant's corresponding British Patent 185,555, accepted Sept. 14, 1922, in which the structural diagrams and a method of manufacture, of each substance, is set forth.

The salts of these tetrazole combinations have various advantages over the known initial bodies and priming agents, among which may especially be mentioned the property to be stored for any length of time without deterioration. It is already known from the literature on this subject that the tetrazole ring is very stable against oxidizing agents and is only split up by concentrated mineral acids at high temperatures. The heavy metal salts of the tetrazoleazoimids, for instance, are therefore scarcely attacked by strong acids or strong lyes, in contradistinction to the ease with which heavy metal azides are attacked.

The new explosives which also have the advantage that they can sustain high pressures without injury and can be formed into pressed bodies are, for instance, in the manufacture of blasting cartridges, mixed with one another or with known explosives or priming ingredients as addition.

As an example, for a charge for blasting cartridges the following may be used:

1.00 g. tetranitromethylaniline (tetryl),  
0.15 g. lead- or cadmium-tetrazylazide,  
0.15 g. azotetrazole lead.

An increase in the safety of handling the tetrazole derivatives which have an extremely high piercing force may be obtained in any known manner, as for instance by granulating them with paraffine or resin dissolved in benzol, xylol, carbon tetrachloride or the like, if desired, and with an admixture of cork-meal, if desired.

In order to combine the valuable properties of different bodies as, for instance, high sensitiveness to ignition, a good power of transmitting flames, a greater specific gravity and in order to obtain in this way universal primers or detonators which can be used for blasting cartridges as well as for Flobert ammunition, it has proved suitable not only to mix the salts of the above named derivatives of tetrazole with other explosives here in question in a mechanical way, but to precipitate them together from solutions, or to crystallize the one salt to the other so as to obtain combinations of salts of the variety of compound crystals or double salts. Difficultly soluble salts of the azoimid, of simply or repeatedly nitrated phenols or their substitution products as, for instance, di- and trinitroresorcin, trinitroorcin and trinitrophloroglucine are well suited for such explosives. Salts of

110

other nitro-bodies possessing favorable properties for the above mentioned primers or detonators are also fit for the manufacture of such compound crystals respecting 5 universal primers or detonators as, for instance, salts of the m-dinitro-o-dinitroso-benzol and trinitro-dinitroso  $\beta$ -naphthol.

The eminently useful chemical properties of the tetrazole compounds as blasting 10 agents have not been known hitherto. Especially the fact that even the smallest quantities of the most explosive of these bodies for instance, tetrazylazides have an excellent initiating action, has never before 15 been found out. It has now been ascertained that of these substances 1 to 2 milligrams are sufficient to bring nitro-pentaerythrit to full detonation. They thus surpass fulminate of mercury in their ignition 20 initiating action to a quite extraordinary degree. Other tetrazole bodies as, for instance, the salts of the azotetrazole also have an advantage over the known explosives as they are of a clear yellow colour, 25 but do not themselves produce a stain. Furthermore in their piercing force they also surpass the salts of known nitro-bodies, as lead trinitroresorcinate and others, which can only be made light coloured 30 with great difficulty, which is a disadvantage in their manufacture and application.

The application of tetrazole derivatives for the manufacture of primers or detonators is entirely new. In the literature only the alkali salts and the silver salt are described, while for the practical application in the arts, the lead and cadmium salts are 35 of main importance.

Tetrazole and its derivatives can equally well be used for Flobert cartridges and 40 similar ammunition in which the primer or detonator acts at the same time as the propelling agent, and also for liquid air cartridges and similar munitions. The ordinary phlegmatizing agents may also be 45 added.

Detonating fuses with the usual wrappings may be manufactured according to this invention by charging ordinary fuses with the salts of tetrazole or its derivates 50 either by themselves or mixed together or mixed with other explosives, if desired, together with a suitable phlegmatizing agent.

What I claim as my invention and desire to secure by Letters Patent is: 55

1. A priming composition for detonating purposes comprising a salt of tetrazole.
2. A priming composition for detonating purposes comprising a salt of a tetrazole derivative. 60

In testimony whereof I affix my signature.

HANS RATHSBURG.